

# UNITED STATES PATENT OFFICE.

GEORGE FRANKLIN ALLEN, OF GRANITE CITY, ILLINOIS, ASSIGNOR TO  
EDWARD R. HOYT, OF ST. LOUIS, MISSOURI.

## ALLOY.

No. 839,444.

Specification of Letters Patent.

Patented Dec. 25, 1906.

Application filed October 24, 1906. Serial No. 340,245.

*To all whom it may concern:*

Be it known that I, GEORGE FRANKLIN ALLEN, a citizen of the United States, residing in Granite City, in the county of Madison, son and State of Illinois, have invented certain new and useful Improvements in Alloys, of which the following is a full, clear, and exact description.

My invention relates to an alloy of metal; and it has for its object to produce an alloy of such nature that it will resist greater tensile strain than other soft-metal alloys; also, an alloy that will be much less subject to corrosion than those heretofore made so far as I am aware.

My alloy consists of three metals—lead, nickel, and copper—combined in such proportions as will cause the nickel and copper to increase the tensile strength of the alloy to the desired degree and will afford the desired

property of lessening the corrodibility of the alloy.

The proportions in which the metals are used vary according to the nature of the lead used, and are from one-twentieth of one per cent. to four and one-half per cent. nickel and from one-twentieth of one per cent. to four and one-half per cent. copper and the balance lead, and preferably soft lead.

I claim—

An alloy consisting of from one-twentieth of one per cent. to four and one-half per cent. nickel, from one-twentieth of one per cent. to four and one-half per cent. copper, and the balance of lead.

GEORGE FRANKLIN ALLEN.

In presence of—

NELLIE V. ALEXANDER,  
BLANCHE HOGAN.